



US008336885B2

(12) **United States Patent**  
**Freling**

(10) **Patent No.:** **US 8,336,885 B2**  
(b5) **Date of Patent:** **\*Dec. 25, 2012**

(54) **WEAR-RESISTANT COATING**(75) Inventor: **Melvin Freling**, West Hartford, CT (US)(73) Assignee: **United Technologies Corporation**,  
Hartford, CT (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/456,658**(22) Filed: **Apr. 26, 2012**(65) **Prior Publication Data**

US 2012/0205874 A1 Aug. 16, 2012

**Related U.S. Application Data**

(62) Division of application No. 13/164,131, filed on Jun. 20, 2011, now Pat. No. 8,187,989, which is a division of application No. 11/376,455, filed on Mar. 15, 2006, now Pat. No. 7,985,703.

(51) **Int. Cl.****F16J 15/34** (2006.01)(52) **U.S. Cl.** ..... **277/404; 277/405**(58) **Field of Classification Search** ..... **277/404-406**  
See application file for complete search history.(56) **References Cited**

## U.S. PATENT DOCUMENTS

|               |        |              |         |
|---------------|--------|--------------|---------|
| 3,751,049 A * | 8/1973 | Busby et al. | 277/382 |
| 3,954,479 A   | 5/1976 | Jahn         |         |
| 4,728,448 A   | 3/1988 | Sliney       |         |

|                 |         |                              |
|-----------------|---------|------------------------------|
| 4,883,639 A     | 11/1989 | Adlerborn et al.             |
| 5,122,182 A     | 6/1992  | Dorfman et al.               |
| 5,536,022 A     | 7/1996  | Sileo et al.                 |
| 5,709,936 A     | 1/1998  | Besmann et al.               |
| 5,763,106 A     | 6/1998  | Blanchard et al.             |
| 5,780,116 A     | 7/1998  | Sileo et al.                 |
| 5,932,356 A     | 8/1999  | Sileo et al.                 |
| 6,132,175 A     | 10/2000 | Cai et al.                   |
| 6,257,589 B1 *  | 7/2001  | Flaherty et al. .... 277/400 |
| 6,607,782 B1    | 8/2003  | Malshe et al.                |
| 2002/0119338 A1 | 8/2002  | Hasz et al.                  |
| 2004/0142196 A1 | 7/2004  | Hajmrle et al.               |

## FOREIGN PATENT DOCUMENTS

|    |             |        |
|----|-------------|--------|
| DE | 19700835 A1 | 7/1997 |
| JP | 59029819 A  | 2/1984 |
| JP | 8117984 A   | 5/1996 |

## OTHER PUBLICATIONS

Official Search Report of the European Patent Office in foreign Application No. 07250918.5, filed Mar. 6, 2007.  
Communication Pursuant to Article 94(3) EPC from European Patent Application No. 07250918.5, filed Mar. 6, 2007.

\* cited by examiner

Primary Examiner — Vishal Patel

(74) Attorney, Agent, or Firm — Kinney &amp; Lange, P.A.

(57) **ABSTRACT**

A seal assembly for a gas turbine engine includes a first seal member having a first surface, a second seal member having a second surface, with the second surface configured to generally abut at least a part of the first surface. At least a portion of at least one of the first surface and the second surface includes a coating that includes about 30 to about 80 weight percent of a hard carbide material, and about 20 to about 70 weight percent of lubricating material incorporated with the hard carbide material. The coating defines overlapping lenticular particles.

**14 Claims, 1 Drawing Sheet**



## 1

## WEAR-RESISTANT COATING

## CROSS-REFERENCE TO RELATED APPLICATION(S)

The present application is a divisional application from U.S. patent application Ser. No. 13/164,131, filed Jun. 20, 2011, which is a divisional from U.S. patent application Ser. No. 11/376,455 (now U.S. Pat. No. 7,985,703), filed Mar. 15, 2006, both of which are herein incorporated by reference in their entireties.

## BACKGROUND

The present invention relates generally to a coating. More particularly, the present invention relates to a coating suitable for use as a wear-resistant coating for a gas turbine engine component.

A wear-resistant coating is often applied to a component that is subject to high friction operating conditions. For example, a gas turbine engine component, such as a seal plate in a rotary seal mechanism, is often subject to high friction and high temperature operating conditions. After some time in service, the friction typically causes the surface of the component that is exposed to the friction to wear. The wear is generally undesirable, but may be especially undesirable and problematic for a sealing mechanism that acts to segregate two or more different compartments of the gas turbine engine. For example, if a sealing component wears (or erodes) and is no longer effective, fluid from one compartment may leak into another compartment. In some portions of a gas turbine engine, failure of the seal mechanism is detrimental to the operation of the gas turbine engine. In those cases, the gas turbine engine must be removed from service and repaired if a part of the seal mechanism wears to the point of seal failure.

A rotary seal mechanism separates two compartments of the gas turbine engine. A rotary seal mechanism typically includes a first component formed of a hard material, such as a carbon seal, that at least in part contacts a surface of a second component formed of a softer material, such as a seal plate, in order to segregate two or more compartments. In some applications, the seal plate rotates as the carbon seal remains fixed, while in other applications, the carbon seal rotates as the seal plate remains fixed. As the seal plate and carbon seal contact one another, the operating temperature and friction levels of both components increase. This may cause the seal plate and/or carbon seal to wear and deteriorate. The relative vibration between the seal plate and the carbon seal during the gas turbine engine operation may also cause frictional degradation and erosion of the seal plate.

It is important to minimize the wear of the seal plate in order to help prevent the rotary seal mechanism from failing. In order to mitigate the wear and deterioration of the seal plate and extend the life of the seal plate, a wear-resistant coating may be applied to the surface of the seal plate that contacts the carbon seal. However, it has been found that many existing wear-resistant coatings crack and spall under the increasingly high engine speeds and pressures. Regardless of the application, it is desirable to increase the life of a wear-resistant coating. Thus, it is also generally desirable to increase the life of wear-resistant coatings that are applied to components other than gas turbine engine components.

## SUMMARY

A seal assembly for a gas turbine engine according to the present invention includes a first seal member having a first

## 2

surface, a second seal member having a second surface, with the second surface configured to generally abut at least a part of the first surface. At least a portion of at least one of the first surface and the second surface includes a coating that includes about 30 to about 80 weight percent of a hard carbide material, and about 20 to about 70 weight percent of lubricating material incorporated with the hard carbide material. The coating defines overlapping lenticular particles.

## BRIEF DESCRIPTION OF THE DRAWINGS

The sole FIGURE is a partial cross-sectional view of a rotary seal, which includes a carbon seal and a seal plate.

## DETAILED DESCRIPTION

The present invention is both a coating suitable for use as a wear-resistant coating for a substrate and a method for coating a gas substrate with the inventive coating. A "substrate" is generally any underlying component, including gas turbine engine components. A coating in accordance with the present invention includes about 20 to about 70 percent of a lubricating material and about 30 to about 80 percent of a hard carbide material. The lubricating material includes, but is not limited to, polytetrafluoroethylene, molybdenum disulfide, boron nitride, cobalt oxide, graphite, and combinations thereof. The hard carbide material includes, but is not limited to, tungsten carbide, silicon carbide, nickel chrome/chromium carbide, titanium carbide, and combinations thereof.

The wear-resistant coating of the present invention is particularly suitable for applying onto a surface of a gas turbine engine component that is subject to high friction operating conditions, such as a seal plate of a rotary seal mechanism. However, the coating may be used with any suitable substrate that is subject to wearing conditions, including other gas turbine engine components having a hard-faced mating surface. It is believed that the inventive coating bonds to many substrate materials, including steel and nickel alloys, without the use of a bond coat. However, in embodiments, any suitable bond coat known in the art may be employed, if desired.

As turbine engine speeds and pressures have increased in order to increase engine efficiency, it has been found that many existing wear-resistant coatings that include a hard carbide material, such as nickel chrome/chromium carbide, crack and spall, as well as undergo excessive degradation under the increasingly strenuous operating conditions. Such cracking and spalling is undesirable and may shorten the life of the component on which the wear-resistant coating is applied. At the very least, the early failure of the wear-resistant coating causes the component to be prematurely removed from service in order to repair the wear-resistant coating.

The life of a hard carbide wear-resistant coating may be increased by incorporating a lubricating material into the coating in an amount sufficient enough to decrease the coefficient of friction of the wear-resistant coating. The percentage of the lubricating material varies from about 20 percent to about 70 percent, depending upon the type of hard carbide material in the coating, as well as the particular application of the wear-resistant coating. The presence of a lubricating material in the wear-resistant coating lowers the coefficient of friction of the coating, which allows the coating to wear slower than many existing hard carbide wear-resistant coatings. Also as a result of the lower coefficient of friction of the coating, less frictional heat is generated between the coating and the component the coating is engaged with. This also decreases the rate of wear of the coating.

The coating of the present invention may be applied to a substrate with any suitable method, such as thermal spraying, including plasma spraying and a high-velocity oxy-fuel (HVOF) thermal spray process. In the embodiment discussed below, a HVOF type of thermal spray process is used. In a HVOF thermal spray process, a high velocity gas stream is formed by continuously combusting oxygen and a fuel. A powdered form of the coating is then injected into the high velocity gas stream. The coating is heated to near its melting point, accelerated, and directed at the substrate to be coated. A coating applied with a HVOF process results in a dense coating. This is partially attributable to the overlapping, lenticular particles (or "splats") of coating material that are formed on the substrate. A coating applied with a HVOF process is applied in compression, rather than tension, which also contributes to the increased density and hardness values as compared to other coating application methods.

A coating of the present invention is preferably applied in a thickness of about 0.0508 millimeters (about 2 mils) to about 0.508 millimeters (about 20 mils). In an embodiment of the present invention, the lubricating material and the hard carbide material are blended prior to applying the materials onto a substrate or co-sprayed onto the substrate through two separate powder feeders. The resulting wear-resistant coating is a uniform layer of the blended lubricating and hard carbide material.

The sole FIGURE is a partial cross-sectional view of a typical gas turbine engine sealing mechanism 10. Sealing mechanism 10 includes an annular carbon seal ring 12, which is carried by seal carrier 14, and an annular seal plate 16, which is carried by rotating shaft 18. Sealing mechanism 10 is an example of a seal that may be used in a bearing compartment of a gas turbine engine to limit leakage of fluid, such as lubricating oil, from compartment 20 into other parts of the gas turbine engine. Carbon seal ring 12 is formed of a carbonaceous material and seal plate 16 is formed of a metal alloy, such as steel, a nickel alloy, or combinations thereof.

Seal carrier 14 biases face 12A of carbon sealing ring 12 against face 16A of seal plate 16. The biasing is accomplished by any suitable method known in the art, such as by a spring force. Shaft 18 carries seal plate 16, and as shaft 18 rotates, seal plate 16 engages with a surface of carbon seal 12 and frictional heat is generated, causing wear problems at the interface of seal plate 16 and carbon seal 12 (i.e., where face 12A of carbon seal contacts face 16A of seal plate 16).

In order to limit leakage of fluid from compartment 20, it is important to maintain contact between face 12A of carbon seal 12 and face 16A of seal plate 16. Yet, such contact causes seal plate 16 and/or carbon seal 12 to wear. In order to help maintain the functionality of the gas turbine engine, it is important for sealing mechanism 10 to withstand the high-speed conditions and high-temperatures generated as a result of the high-speed conditions. Coating 17, which incorporates a lubricating material and a hard carbide material in accordance with the present invention, is applied to at least a part of face 16A of seal plate 16 that contacts face 12A of carbon seal 12 (coating 17 is not drawn to scale in FIGURE). Coating 17 helps prevent erosion and deterioration of face 16A of seal plate 16 that results from contacting face 12A of carbon seal 12 (e.g., from friction), which helps prevent seal mechanism 10 from failing. Carbon seal 12 is formed of a harder and more wear-resistant material than seal plate 16, and the rate of wear is slower for carbon seal 12 than it is for seal plate 16.

In the embodiment of the FIGURE, coating 17 is applied with a HVOF thermal spray process in a thickness of about 0.0508 millimeters (about 2 mils) to about 0.508 millimeters (about 20 mils).

In embodiments, the carbon seal 12 may be coated with coating 17, either in addition to or instead of coating the seal plate 16 with coating 17.

Sealing mechanism 10 is shown as a general example of a component (or substrate) that includes surfaces subject to wearing conditions. A coating in accordance with the present invention is also suitable for applying to components other than gas turbine engine components that are exposed to wearing conditions, such as the mating face of flanges.

The terminology used herein is for the purpose of description, not limitation. Specific structural and functional details disclosed herein are not to be interpreted as limiting, but merely as bases for teaching one skilled in the art to variously employ the present invention. Although the present invention has been described with reference to preferred embodiments, workers skilled in the art will recognize that changes may be made in form and detail without departing from the spirit and scope of the invention.

While the invention has been described with reference to an exemplary embodiment(s), it will be understood by those skilled in the art that various changes may be made and equivalents may be substituted for elements thereof without departing from the scope of the invention. In addition, many modifications may be made to adapt a particular situation or material to the teachings of the invention without departing from the essential scope thereof. Therefore, it is intended that the invention not be limited to the particular embodiment(s) disclosed, but that the invention will include all embodiments falling within the scope of the appended claims.

The invention claimed is:

1. A seal assembly for a gas turbine engine, the seal assembly comprising:

a first seal member including a first surface; and  
a second seal member including a second surface, wherein  
the second surface is configured to generally abut at least  
a part of the first surface,  
wherein at least a portion of at least one of the first surface  
and the second surface includes a coating comprising:  
about 30 to about 80 weight percent of a hard carbide  
material; and  
about 20 to about 70 weight percent of lubricating mate-  
rial incorporated with the hard carbide material,  
wherein the coating defines overlapping lenticular  
particles.

2. The seal assembly of claim 1, wherein the hard carbide  
material is selected from a group consisting of nickel chrome  
and chromium carbide, tungsten carbide, silicon carbide, tit-  
anium carbide, and combinations thereof.

3. The seal assembly of claim 1, wherein the lubricating  
material is selected from a group consisting of polytetrafluoro-  
ethylene, boron nitride, cobalt oxide, and combinations  
thereof.

4. The seal assembly of claim 1, wherein the lubricating  
material comprises cobalt oxide.

5. The seal assembly of claim 1, wherein the lubricating  
material is selected from a group consisting of polytetrafluoro-  
ethylene, molybdenum disulfide, boron nitride, cobalt  
oxide, graphite, and combinations thereof.

6. The seal assembly of claim 1, wherein the hard carbide  
material and lubricating material are co-sprayed onto the  
second surface of the second seal member.

7. The seal assembly of claim 1, wherein the hard carbide  
material and lubricating material are blended together prior to  
being applied onto at least a portion of at least one of the first  
surface and the second surface.

8. A seal assembly for a gas turbine engine, the seal assem-  
bly comprising:

**5**

a first seal member including a first surface; and a second seal member including a second surface, wherein the second surface is configured to generally abut at least a part of the first surface,  
 wherein at least a portion of at least one of the first surface and the second surface includes a coating consisting essentially of:  
 about 30 to about 80 weight percent of a hard carbide material; and  
 about 20 to about 70 weight percent of lubricating material incorporated with the hard carbide material, wherein the coating defines overlapping lenticular particles.

9. The seal assembly of claim 8, wherein the hard carbide material is selected from a group consisting of nickel chrome and chromium carbide, tungsten carbide, silicon carbide, titanium carbide, and combinations thereof.

**6**

10. The seal assembly of claim 8, wherein the lubricating material is selected from a group consisting of polytetrafluoroethylene, boron nitride, cobalt oxide, and combinations thereof.
- 5 11. The seal assembly of claim 8, wherein the lubricating material comprises cobalt oxide.
12. The seal assembly of claim 8, wherein the lubricating material is selected from a group consisting of polytetrafluoroethylene, molybdenum disulfide, boron nitride, cobalt oxide, graphite, and combinations thereof.
- 10 13. The seal assembly of claim 8, wherein the hard carbide material and lubricating material are co-sprayed onto the second surface of the second seal member.
- 15 14. The seal assembly of claim 8, wherein the hard carbide material and lubricating material are blended together prior to being applied onto at least a portion of at least one of the first surface and the second surface.

\* \* \* \* \*